

## UNITED STATES PATENT OFFICE.

ELBRIDGE B. FULKS, OF LOUISVILLE, KENTUCKY, ASSIGNOR TO THE AMERICAN CREOSOTING COMPANY, OF LOUISVILLE, KENTUCKY, A CORPORATION OF INDIANA.

## METHOD OF PRESERVATIVELY TREATING WOODS.

No Drawing.

Application filed January 9, 1926. Serial No. 80,358.

This invention relates to a method of preservatively treating woods.

In the usual method of preparing timbers for treatment with creosote the moisture is extracted either by air seasoning or by heating with live steam in a closed cylinder, after which the usual vacuum is created for the removal of sufficient moisture. A preservative such as creosote is maintained in the usual manner in close association with the fluid until full sap penetration is had. However, this process results in a great waste of the preservative because an excess of creosote is always required.

It is also necessary to classify timbers with respect to certain physical characteristics such as their ability to absorb the preservative. Even under the well known methods of classification of timber as to their relative absorption qualities, it will be found that some pieces under treatment with a preservative have absorbed a greater proportion of the preservative than others, while certain of the timbers have absorbed the preservative with considerable difficulty. It will be readily seen that in order to obtain a satisfactory impregnation of the pieces of timbers which tend to absorb the preservative with difficulty it is necessary to use high pressure for a considerable length of time with a consequence that the pieces of timber which are more susceptible to the absorption of the preservative contain the preservative in a quantity which is in excess of the amount required. When the preservative employed is creosote oil, the waste is expensive.

It is an object of the present invention to provide a treatment for the timbers in advance of the final preservative treatment which will create a uniform state of resistance in the woods to the impregnation of creosote so that all of the timbers when treated with creosote oil will have a substantially uniform saturation of the oil.

A further object of the invention is the provision of a method of treating woods in which the resistance to the impregnation of the creosote oil is determined by the saturation of the timbers with a liquid or weak solution of a salt in advance of the treatment of the creosote oil so that when the oil is supplied under pressure the timbers will not absorb a greater quantity of the creosote than is necessary for the purpose.

A still further object of the invention is the provision of a process in which timbers of varying degrees of susceptibility to liquid penetration are treated either with water or a toxic salt, such for example, as a weak solution of zinc chloride until the timbers are sufficiently saturated with either of these elements so that an excess impregnation of a creosote oil at the final treatment will be prevented.

This invention will be best understood from a consideration of the following detailed description; nevertheless it is to be understood that the invention is not confined to the disclosure, being susceptible of such changes and modifications which shall define no material departure from the salient features of the invention as expressed in the appended claims.

In carrying out my invention the timbers are selected in the usual manner and classified and then segregated. A charge of the timbers having approximately the same degree of absorptive capacity for a preservative are given the usual preliminary treatments, including the subjection of the wood to live steam under pressure in a closed vessel. The charge of the classified timbers having varying degrees of moisture content are placed in a drum or any closed vessel and are then saturated in any well known manner with a preliminary treatment of the liquid. This liquid may be any ingredient which will partially saturate the timbers sufficiently to provide a predetermined degree of resistance to the impregnation of a toxic ingredient such as creosote oil.

It is found that water, water vapor or steam, provide very suitable commercial fluids for the purpose. However, certain advantages are gained by the use of a weak solution of a toxic salt and since zinc chloride affords a cheap toxic salt, a solution of this salt may be employed for the saturation of the timbers.

While I have stated that zinc chloride is employed because of its cheapness, such other salts as, sodium or potassium arsenate, sodium chloride or copper sulphate may be used in the preliminary treatment.

By such a treatment all of the timbers have substantially the same degree of penetration because of the fact that water in any form or a toxic salt solution has previously penetrated the timbers and remains therein,

thereby providing for approximately an equalized resistance to the permeability of the creosote solution. The purpose of the preliminary liquid treatment is to bring 5 each of the timbers, regardless of its characteristics, to its saturation point for aqueous liquids. The result is that a predetermined quantity of the creosote solution is only required for an efficient preservative treatment 10 so that a great quantity of the preservative which was formerly wasted by excess penetration will be saved, as the body of liquid within the timbers prevents any excess.

15 Certain timbers such as pine have areas of greater resistance to the creosote and when such timbers are treated preliminarily with water or the toxic salt solution, the less resistant portions of the timbers are sufficiently saturated so that there will be created 20 in such timbers a uniform state of resistance to the impregnation of creosote.

25 In the ordinary treatment of timber with creosote, the time required is from about thirty minutes for easily treated timbers, to five or six hours for more refractory timbers. The time required to treat timbers with water or liquid solution of toxic salt would be from thirty minutes to two or three hours, so that the total time required for 30 this process, might be from forty-five minutes to seven or eight hours.

35 Heretofore in the art of preservatively treating woods it has been customary first to fill the pores of the wood with a toxic salt solution and then to extract the solution upon the theory that some salt will be deposited within the wood, but leaving however, the pores open as before. In consequence, when the final creosote treatment is given, there is 40 nothing filling the internal cells of the timbers with which to prevent the highly expensive excess penetration of creosote. In my process the preliminary treatment liquid is retained within the wood, excepting that a 45 small amount is withdrawn from the surface area under the conventional vacuum treatment, and the creosote then applied under pressure. As it is immiscible with water, its penetration beyond a certain point is 50 positively checked.

After the wood has been impregnated with creosote under pressure, the pressure is preferably released and the surplus creosote removed while the wood is maintained under

55 a vacuum, after which the wood is subjected to a quick high vacuum.

What I claim is:

1. A process for preservatively treating wood which comprises impregnating the wood with water in such manner as to resist 60 the flow of a preservative liquid and then impregnating the water saturated wood a predetermined depth with creosote.

2. A process for preservatively treating wood which comprises impregnating wood 65 with a solution of a toxic salt in such manner as to retain the solution therein, and then impregnating the wood with creosote.

3. A process for preservatively treating wood which comprises subjecting wood to 70 live steam under pressure in a closed vessel, then subjecting wood to a solution of a toxic salt under pressure, removing only the surplus solution of the toxic salt, then subjecting the wood to creosote under pressure.

75 4. A process for preservatively treating wood which comprises subjecting wood to live steam under pressure in a closed vessel, then subjecting wood to a solution of a toxic salt under pressure, removing the surplus solution of the toxic salt, then subjecting the wood to creosote under pressure, releasing the pressure and removing the surplus creosote while maintaining the wood under a vacuum, and then subjecting the wood to a 85 quick high vacuum.

90 5. A step in the process for preservatively treating wood which comprises saturating a plurality of pieces of wood which are susceptible of varying degrees of impregnation by a creosote oil, with an aqueous liquid until the pieces of wood have become susceptible to the same degree of impregnation of the creosote oil, then treating the wood with creosote oil.

95 6. A process for preservatively treating wood which comprises forcing creosote under pressure into wood initially saturated with an aqueous liquid, against the retained liquid.

100 7. A process for preservatively treating wood which comprises forcing a preservative under pressure into wood initially saturated with an aqueous liquid, against the retained liquid, said preservative and aqueous liquid being naturally immiscible.

105 In testimony whereof I affix my signature.  
ELBRIDGE B. FULKS.